

## UNITED STATES PATENT OFFICE.

JAMES W. SCHWAB, OF GULF, TEXAS, ASSIGNOR TO TEXAS GULF SULPHUR COMPANY, OF BAY CITY, TEXAS, A CORPORATION OF TEXAS.

## CASTING SULPHUR.

No Drawing.

Application filed November 2, 1923. Serial No. 672,445.

To all whom it may concern:

Be it known that I, JAMES W. SCHWAB, a citizen of the United States, residing at Gulf, in the county of Matagorda, State of Texas, have invented certain new and useful Improvements in Casting Sulphur; and I do hereby declare the following to be a full, clear, and exact description of the invention, such as will enable others skilled 10 in the art to which it appertains to make and use the same.

This invention relates to the solidification or casting of molten sulphur, and has for its object the provision of certain improvements 15 in casting sulphur whereby the sulphur is rendered easily parted from the surface against which it solidifies.

In the production or mining of sulphur by underground fusion, for example, in accordance 20 with the well known Frasch process, a fusing fluid, such as superheated water, is conveyed to the underground sulphur deposit where its heat is utilized in fusing the sulphur and the fused sulphur 25 is raised to the surface of the ground in a molten condition by suitable agencies, such as an air lift pump.

The satisfactory disposition of the molten sulphur as it is discharged at the surface of 30 the ground from the so-called sulphur wells presents certain peculiar difficulties. At the present time, it is the customary practice to solidify the sulphur in the form of a huge block or pile containing many thousands 35 of tons of sulphur. Thus, in accordance with the present prevailing practice, the molten sulphur is conveyed from the sulphur wells to a bin made up of four enclosing walls extending an appropriate distance 40 above the ground level. The enclosing walls are frequently several hundred feet in length and are designed to hold or enclose a huge quantity of sulphur. The molten sulphur flows into this bin or 45 closure and eventually solidifies into a huge block or pile. In actual practice, many weeks and frequently months elapse before this block of sulphur becomes solid throughout its entire mass.

50 The block or pile of sulphur, formed as above described, must be broken up for the subsequent handling and shipment from the sulphur field to the consumer. To this end, it is necessary to blast the sulphur pile in 55 substantially the same manner that rock is

blasted. By repeated blasting and considerable manual labor, the sulphur is finally prepared for loading, usually by automatic loading machinery, into freight cars or other conveyances of transportation. The 60 present practice of solidifying the molten sulphur thus involves the formation of a huge pile of solid sulphur and the subsequent breaking up of this pile of sulphur into suitable form for convenient handling 65 and transportation. The present practice in this respect necessitates the provision above ground of an enormous quantity of sulphur since while one pile or block of sulphur is being broken down and shipped, 70 another block must be in process of formation, and on this account many thousands of tons of sulphur are constantly maintained above ground. This is obviously an 75 uneconomical procedure and it is extremely desirable that a more rapid method of solidifying sulphur be provided by which the molten sulphur may be prepared for shipment within a relatively short time after it is discharged from the sulphur wells, thereby 80 reducing the amount of sulphur which must be accumulated above ground.

From an operating standpoint the most suitable rapid methods of solidification are those which cast the sulphur in relatively 85 small cakes in a pan conveyor or in large cakes by building up such cakes in thin layers on a belt conveyor.

One of the greatest operating drawbacks to these methods of rapid solidification is 90 the difficulty with which solid sulphur is freed from the mold or belt upon which it has solidified. Efforts have been made to overcome this tendency of the sulphur to cling to the surfaces against which it 95 solidifies by the application of exterior means, such as moistening the inner surfaces of the mold with water or other liquids and at the same time allowing the mold to rest in water. Under proper conditions this results in such rapid cooling of a thin layer of sulphur next the sides and bottom of the mold that the water inside the mold is not evaporated by the heat from the sulphur but remains as a thin film and 100 keeps the sulphur from adhering to the mold. But if the inner surface of the mold is not entirely wetted the sulphur comes into direct contact with the surface of the mold in that portion which is not wetted 105 110

and may stick to the mold. In many cases it clings so tenaciously to the molds that the solid cake must be laboriously broken out in small pieces by hand. If there is 5 too much water in the mold some of it may become enclosed in the solid sulphur and greatly increase the moisture content of the product.

In contradistinction to these efforts to 10 overcome the tendency of sulphur to cling to the surfaces against which it solidifies, I have discovered that sulphur may be rendered easily removable from the molds in which it is cast by subjecting the molten 15 sulphur to a preliminary treatment with an appropriate agent for modifying the properties of the sulphur so as to eliminate in large part its tendency to cling to the surface of a mold, while the sulphur is not 20 harmed or rendered unfit for commercial uses. Thus, if molten sulphur is brought in intimate contact with a small amount 25 of certain alkaline substances, such as ammonia, for a sufficient time to allow the alkaline substance to react with the sulphur, it may be readily and easily removed from the molds in which it is solidified or cast. Preferably, the thus treated sulphur should be cast as soon as possible after 30 treatment.

In accordance with my preferred practice 35 of the invention, I subject molten sulphur to an appropriate preliminary treatment with ammonia whereby the ammonia is brought in intimate contact with the molten sulphur for a sufficient time for the sulphur to take up the ammonia. The ammonia may be added to the sulphur in any convenient manner. In order to conserve ammonia it is best 40 to agitate the liquid sulphur with the required amount of ammonia in a closed tank. A similar result may be obtained by other means such as circulating the ammonia through the liquid sulphur in a closed tank 45 by means of a pump or blower, or, if conditions permit, by simply bubbling the ammonia through the liquid sulphur in an open tank and allowing the excess ammonia to escape. The sulphur should be cast as soon 50 as possible after treatment.

The amount of ammonia required to bring about the desired result varies somewhat with the sulphur. Good results may be obtained when treating Frasch process 55 sulphur with from about 0.023 pound to about 0.09 pound of ammonia per long ton of sulphur. In some cases an even smaller amount of ammonia may be sufficient.

The duration of treatment or the period 60 of contact between the liquid sulphur and ammonia may vary somewhat with the quantity of sulphur being treated and the method employed for bringing about the intimate contact between the sulphur and ammonia. 65 I have secured satisfactory results when

treating small quantities of sulphur by agitating the mixture of ammonia and sulphur for about one minute.

The temperature at which treatment and subsequent pouring into molds takes place 70 has little effect upon the final result although the more nearly the sulphur approaches the temperature of its solidification point and the cooler the mold, the more rapidly the solidification and parting from 75 the mold. In actual practice the sulphur can best be handled at the temperature ordinarily used for transporting liquid sulphur, namely, about 130-140° C. The length of time required for cooling the cast sulphur 80 may be materially shortened by making use of any of the well known expedients for this purpose, such, for example, as allowing the outside surface of the mold to dip into water. 85

Investigations were made to determine the actual amount of ammonia required and to show by comparison with untreated sulphur the greater rapidity with which ammonia treated sulphur parts from the mold. In making the experiments small quantities of liquid ammonia were sealed in glass tubes and weighed. A tube containing a known weight of ammonia was dropped into a flask containing a weighed amount of liquid sulphur. The flask was quickly stoppered and shaken. The glass tube was broken by the great increase in pressure and the ammonia vaporized instantaneously. The flask containing this mixture of sulphur and ammonia was then shaken continuously for about one minute so that the sulphur and ammonia came into intimate contact. The sulphur was then poured into a mold and the time required for the sulphur to part 100 from the mold noted. Glass molds were used so that the parting of the sulphur from the mold could be more easily observed. 105

Typical results of these investigations are given in the following tables. Table No. 1 110 gives the results obtained by casting sulphur which has been subjected to a preliminary treatment in accordance with the invention, and Table No. 2 gives results obtained when casting untreated sulphur. 115

No. 1

| Lbs.<br>ammonia<br>per long<br>ton of<br>sulphur | Temperature in<br>degrees C. |                    | Mold<br>water<br>cooled | Time<br>to<br>part<br>from<br>mold | Remarks                          | 120 |
|--------------------------------------------------|------------------------------|--------------------|-------------------------|------------------------------------|----------------------------------|-----|
|                                                  | During<br>treatment          | At<br>pour-<br>ing |                         |                                    |                                  |     |
| 0.09                                             | 122                          | 122                | No....                  | 20 sec....                         |                                  |     |
| 0.075                                            | 148                          | 136                | No....                  | 5 min....                          | Mold heated to 140° C. at start. | 125 |
| 0.045                                            | 140                          | 120                | No....                  | 15 sec....                         |                                  |     |
| 0.038                                            | 148                          | 136                | No....                  | 5 min....                          |                                  |     |
| 0.03                                             | 145                          | 122                | No....                  | 2 min....                          |                                  |     |
| 0.03                                             | 146                          | 130                | No....                  | 2.5 min....                        |                                  |     |
| 0.03                                             | 146                          | 132                | Yes....                 | 1 min....                          |                                  |     |
| 0.023                                            | 145                          | 125                | No....                  | 2 min....                          |                                  |     |
| 0.023                                            | 145                          | 126                | Yes....                 | 1 min....                          |                                  |     |

No. 2

| 5  | Lbs.<br>ammonia<br>per long<br>ton of<br>sulphur | Temperature in<br>degrees C. |                    | Mold<br>water<br>cooled | Time to part from<br>mold |
|----|--------------------------------------------------|------------------------------|--------------------|-------------------------|---------------------------|
|    |                                                  | During<br>treat-<br>ment     | At<br>pour-<br>ing |                         |                           |
| 10 | None.....                                        |                              | 140                | No.....                 | 20 min.                   |
|    | None.....                                        |                              | 121                | No.....                 | 18 min.                   |
|    | None.....                                        |                              | 124                | Yes.....                | 16 min.                   |

## I claim:

1. The improvement in casting sulphur which comprises subjecting molten sulphur 15 to a preliminary treatment with an alkaline substance for modifying the properties of the sulphur so as to eliminate in large part its tendency to cling to the surface of a mold, and thereafter casting in molds the 20 sulphur thus treated.

2. The improvement in casting sulphur which comprises bringing molten sulphur in intimate contact with ammonia so as to modify the properties of the sulphur to eliminate in large part its tendency to cling 25 to the surface of a mold, and thereafter casting the sulphur in molds.

3. The improvement in casting sulphur which comprises bringing molten sulphur in intimate contact with ammonia at a temperature slightly greater than the temperature of solidification of the sulphur so as to modify the properties of the sulphur to eliminate in large part its tendency to cling 30 to the surface of a mold, and thereafter 35 pouring the sulphur in molds for solidification.

In testimony whereof I affix my signature.

JAMES W. SCHWAB.